# EUROPEAN PATENT SPECIFICATION

(11) **EP 3 083 105 B1**
(45) Date of publication and mention of the grant of the patent: **15.11.2017**
(21) Application number: 14835731.2
(22) Date of filing: 10.12.2014
(51) Int. Cl.: B22D 25/00

(54) **CONTINUOUS COMPOSITE METAL FOAM PRODUCTION AND METHOD AND DEVICE FOR STIRRING PARTICLE REINFORCED COMPOSITE METAL**
KONTINUIERLICHE HERSTELLUNG VON VERBUNDMETALLSCHAUM UND VERFAHREN UND VORRICHTUNG ZUM RÜHREN EINES PARTIKELVERSTÄRKTEN VERBUNDMETALLS
PRODUCTION D'UNE MOUSSE MÉTALLIQUE COMPOSITE CONTINUE ET PROCÉDÉ ET DISPOSITIF PERMETTANT D'AGITER UN MÉTAL COMPOSITE RENFORCÉ PAR DES PARTICULES

(30) Priority: 17.12.2013 TR 201314802
(43) Date of publication of application: 26.10.2016
(73) Proprietor: Taskin, Nilhan Urkmez, Edirne (TR); Taskin, Vedat, Edirne (TR)
(72) Inventor: Taskin, Nilhan Urkmez, Edirne (TR); Taskin, Vedat, Edirne (TR)
(74) Representative: Karaahmet, Erdogan
(86) International application number: PCT/TR2014/000497
(87) International publication number: WO 2015/094139

(56) References cited:
- WO-A1-03/064711
- WO-A2-2008/003290
- DE-A1- 2 218 455
- DE-C1- 4 326 982
- US-A- 5 281 251
- V. Taskin, N.Ü. Taskin, P.A. Demirhan, I. Mutlu: "Manufacturing of composite metal foam by directly foaming at semi solid temperature" In: "Proceedings UNITECH`10 Gabrovo", 2010, Gabrovo, XP002740336, pages II-193-II-196, pages II-194 - pages II-195
- N.Ü. Taskin, V. Taskin, I. Mutlu, P. A. Demirhan: "The effect of reinforcement ratio and heat treatment on compressive behavior of 7075 Al/SiCp composite foam" In: "Proceedings UNITECH`10 Gabrovo", 2010, Gabrovo, XP002740337, pages II-201-II-205, pages II-201 - pages II-202
- RAMIN JAMSHIDI-ALASHTI, MEHDI KASKANI, BEHZAD NIROUMAND: "Semisolid melt squeezing procedure for production of open-cell Al-Si foams", MATERIALS AND DESIGN, vol. 56, 26 November 2013 (2013-11-26), XP002740338,
- Nan Li, Shuming Xing, Peiwei Bao, Zhimin Liu: "A Research on Fabrication of Aluminum Foam Precursor Using Semi-solid Melt" In: "Proceedings ICMEE 2010", 2010, XP002740339, vol. 1 the whole document
- BANHART J: "Aluminium foams for lighter vehicles", INTERNATIONAL JOURNAL OF VEHICLE DESIGN, ST HELIER, GB, vol. 37, no. 2/3, 1 January 2005 (2005-01-01), pages 114-125, XP001525928, ISSN: 0143-3369

## Description

### Technical Field of the Invention

This invention is related to a method and a device that performs said method in order to carry out in one go, the production of closed cell, and continuous form composite metal foam production without the necessity to perform pre-processes thereon; to increase the quality and strength of the material, to distribute the reinforcement and/or foam material homogenously within the material, to be able to produce foam material having the desired density and to provide a homogenous inner structure, moreover, to be able to mix homogenously at the desired ratios, the reinforcement material and the matrix material during the production of particle reinforced composite metal, to distribute the ceramic particles used as reinforcement material into the material homogenously and in order for the material to be wetted better by the matrix material and in order to increase the quality of the material.

### Prior Art related to the art of metal foams

The publications (articles and thesis) within the known state of the art related to the method and device for producing continuous composite metal foam have been listed below.
[1] Ashby, M. F., Evans, A., Fleck, N. A., Gibson, L. J., Hutchinson, J. W. and Wadley, H. N. G., "Metal Foams: A Design Guide", Butterworth-Heinemann Woburn, USA,ISBN 0-7506-7219-6,2000
[2] Wassim Elias Azzi, "A Systematic Study On The Mechanical And Thermal Properties Of Open Cell Metal Foams For Aerospace Applications" Ph.D. Thesis, North Carolina State University, Raleigh, ,2004.
[3] John Banhart, "Manufacture, Characterization and Application of Cellular Metals and Metal Foams" John Banhart & Denis Weaire, "On the road again: Metal foams find favor". Physics Today, 2002.
[4] H.P. Degischer, Handbook of Cellular Materials - Production, Processing, Applications,H.P. Degischer y B. Kriszt (Eds.), Wiley-VCH, Weinheim, pp. 5-7.,2000
[5] Matijasevic-Lux, B. (2006). Characterization and optimization of blowing agent for making improved metal foams, Doctor Eng. Science thesis, Technical University of Berlin
[6] S. Elbir, S. Yilmaz, A. K. Toksoy, M. Guden "SiC-Particulate Aluminum Composite Foams Produced By Powder Compacts: Foaming And Compression Behavior" Journal Of Materials Science 38,4745-4755,2003
[7] S. Esmaeelzadeh A, A. Simchi, "Foamability And Compressive Properties Of AISi7-3 Vol.% SiC-0.5 Wt.% TiH2 Powder Compact", Materials Letters, 2008
[8] Wang Deqing, Shi Ziyuan, "Effect Of Ceramic Particles On Cell Size And Wall Thickness Of Aluminum Foam", Materials Science And Engineering A361,45-49,2003
[9] F. Simancik, L. Lucan And J.Jerz, "Reinforced Aluminium Foams" Institute Of Materials And Machine Mechanics, Sas, Bratislava, Slovak Republic
[10] B.P.Neville,A.Rabiei,"Comp. Metal Foams Processed Through Powder Metallurgy", Mat. And Des.29-388-396,2008
[11] Rabiei, A.T. O'neill, "A Study On Processing Of A Composite Metal Foam Via Casting", Materials Science And Engineering A 404,159-164,2005
[12] Lakshmi J. Vendra, Afsaneh Rabiei, "A Study On Aluminum-Steel Composite Metal Foam Processed By Casting" Materials Science And Engineering A 465,59-67,2007
[13] Banhart, J., Fleck, N. and Mortensen, A., "Cellular Metals: Manufacture, Properties, Applications", Verlag Metall Innovation Technologie MIT Berlin, Germany,ISBN 3-935538-12-X,2003
[14] Ashby,M.F.,"Materials Selection in Mechanical Design",Butterworth-Heinemann Oxford,UK,ISBN 0 7506 6168 2,2005
[15] Stadler, C., Hosnedl, S. and Lasova, V., "Organ Features Incorporating Metal Foams-their Properties and their Relationships and Evaluation", Proc.of the 4th Int. Conf. on Porous Metals and Metal Foaming Tech.-MetFoam05,, Japan, 2005.
[16] John Banhart, Manufacture, "Characterization And Application Of Cellular Metals And Metal Foams", Progress In Materials Science, 46, 559-632, 2001
[17] Esmaeelzadeh,S., Simchi, A., Lehmhus, D., "Effect of Ceramic Particle Addition on the Foaming Behavior, Cell Structure and Mechanical Properties of P/M AISi7 Foam", Materials Science and Engineering, A424, 290-299,2006
[18] Yu, S., Luo, Y., Liu, J., "Effects of Strain Rate and SiC Particle on the Compressive Property of SiCp/AlSi9Mg Composite Foams", Materials Science and Engineering, 487, 394-399,2008
[19] Gui, M.C., Wang, D.B., Wu, J.J., Yuan, G.J., Li, C.G., "Deformation and Damping Behaviors of Foamed Al-Si-SiCp Composite", Materials Science and Engineering, A286, 282-288,2000
[20] Esmaeelzadeh, S., Simchi, A., "Foamability and Compressive Properties of AISi7 - 3 Vol.% SiC- 0.5 Wt.% Tih2 Powder Compact", Materials Letters, 62, 1561-1564,2008
[21] Jeon, Y.P., Kang,C.G., Lee, S.M., "Effects of Cell Size on Compression and Bending Strength of Aluminum-Foamed Material by Complex Stirring in Induction Heating", Journal of Materials Processing Technology, 2 0 9, 435-444,2009
[22] Luo, Y., Yu, S., Li, W., Liu, J., Wei, M., "Compressive Behavior of SiCp/Alsi9Mg Composite Foams", Journal of Alloys and Compounds, 460, 294-298,2009
[23] Yu, C.J., Banhart, J., "Mechanical Properties of Metallic Foams", Fraunhofer USA Metal Foam Symposium, 37-48,1997
[24] Haesche, M., Weise, J., Garcia-Moreno, F., Banhart, J., "Influence of Particle Additions on The Foaming Behaviour of AlSi11/TiH2 Composites Made by Semi-Solid Processing", Materials Science And Engineering, 480, 283-288,2007
[25] Taskin, V., Taskin, N. U., Demirhan, P. A., Mutlu, I., "Manufacturing Of Composite Metal Foam By Directly Foaming At Semi Solid Temperature", Proceedings UNITECH'10 Gabrovo, II-193-II-196, 2010

Metal foams (Metal Foam) can be used in several fields from mechanical applications to thermal applications due to their perfect durability /weight ratios [1-4,13,15]. Metal foams, form interesting physical and mechanical characteristics when high durability is combined with very low specific gravity or high gas permeability is combined with heat treatment conduction.

They are characterized with cell topologies, structurally, or by the fact that they are open or closed cells, according to their specific intensities, to their cell sizes, cell shapes, and anisotropies. They can be produced from different materials such as aluminum, titanium and nickel. As a result the field of application determines the type of material from which the metal foam should be produced from. [4,13].

Due to their low densities, perfect specific durability, noise insulation, and impact and flame damping characteristics, studies that have increased recently especially regarding closed cell Metal Foams in sectors such as space, aviation, and automotives attract attention [3,4]

Mainly two methods are used to produce Metal Foam's which are the liquid phase and the solid phase. The structural and durability characteristics show difference in connection with the production method. There are several studies related to the problems that arise during production. [5-9,16,18-23].

The main problems that are faced during the production of metal foams that are produced using liquid phase methods, are not being able to provide sufficient resistance in the cell walls, not being able to control cell sizes and distribution, combining of cells, and the obligation to perform heat treatment on powders that are used as foaming agents [11-13,21]. In the patent publications numbered US2005161188, HU0800736, WO2006021082, it has been explained that reinforcement material is added into liquid metal prior to the foaming process in order to increase resistance and foam stability and to thicken the walls of cells. This application has been described in the publication numbered WO2008003290.

It is said that that in these studies where composite foam production is carried out, the matrix and reinforcement materials are in contact with each other for a long time and due to this reason unwanted brittle phases occur in inter surfaces, and that homogenously distributing the reinforcement material within the liquid phase is a difficult task on which studies are still being carried out. [6,8-12,17,18].

Although production is possible using liquid phase production methods, due to weak resistance characteristics they have limited usage in structural applications [5,7,8,and 9].

Cell size and distribution control can be relatively carried out in metal foams that have been produced by first forming a preform by means of sintering and then heating in a furnace or in limited volumes; however the product sizes and numbers obtained with these kind of methods are limited (WO2010127668 and WO201010106883). Moreover the sintering procedure is quite long. The precautions taken in order to prevent these kinds of disadvantages also increase process costs. [10,11].

The method and device, developed by means of the present invention, in order to produce a continuous composite metal foam or particle reinforced composite metal overcomes the disadvantages mentioned above and the method and device developed according to the present invention is characterized by the following:
- Closed cell composite foam materials reinforced with ceramic particles added in different ratios can be directly produced using the semi solid production method,
- Ceramic particles and foaming powders are mixed into the semi solid metal or metal alloys,
- The stirring procedure is carried out when the material is semi solid by means of stirrers having different profiles, prepared from graphite rods,
- The semi solid mixture is added to movable molds by means of a piston after the stirring process has been completed,
- The size of the product is determined by the section of the mold and the volume of the crucible,
- Following the foaming procedure that has been carried out inside a furnace the product is taken out of the furnace by means of a pushing mechanism,
- It is quickly cooled by a cooling system located outside of the furnace, and as a result the metal foam production having the desired characteristics is produced.

### KNOWN STATE OF THE ART RELATED TO PARTICLE REINFORCED COMPOSITE METAL

The publications (articles and thesis studies) within the known state of the art related to the method and device for particle reinforced composite metal stirring developed by means of this invention have been listed below.
[1] Naher,S., Brabazon,D., Looney,L, "Development and assessment of a new quick quench stir caster design for the production of metal matrix composites", Journal of Material Processing Technology, 166,430-439.,2004
[2] Zhou, W. and Xu, Z.M., "Casting of SiC reinforced metal matrix composites", J. of Mat. Proc.Tech., 63, 358-363.,1997
[3] D.O.D., "Department of Defense Handbook", Comp. Mat. Handbook, Metal Matrix Composites, Vol.4.,1999
[4] Kaczmar, J.W., Pietrzak, K., Wlosinski, W., "The production and application of metal matrix composite materials", Journal of Materials Processing Technology 106, 58-67,2000
[5] William, C., Harrigan, Jr.,"Commercial processing of metal matrix composites", Mat. Sci. and Eng. A244,75-79,1998
[6] Evans, A., San Marchi, C., Mortensen, A., "Metal Matrix Composites in Industry, An Introduction and a Survey", 440 p., Hardcover, ISBN: 978-1-4020-7521-6,2003
[7] O'Donnell, G., Looney, L., "Production of Aluminium Matrix Composite Components Using Conventional PM Technology", Materials Science and Engineering A303,292-301,2001
[8] Hashim, J. Looney, L., Hashmi, M.S.J,. "The Wettability of SiC Particles by Molten Aluminium Alloy", Journal of Materials Processing Technology 119, 324-328,2001
[9] Hashim, J., Looney,L., Hashmi, M.S.J., "Particle distribution in cast metal matrix composites-Part I", Journal of Materials Processing Technology 123, 251-257,2002
[10] Hashim, J., Looney,L., Hashmi, M.S.J., "Particle distribution in cast metal matrix composites-Part II", Journal of Materials Processing Technology,123 ,258-263,2002
[11] Shi, Z., Ochiai, S. , Gu, M., Hojo, M. and Lee, J.C., "The formation and thermostability of MgO and MgAl2O4 nanoparticles in oxidized SiC particle-reinforced Al-Mg composites", Applied Physics A: Materials·Science & Processing Springer Berlin / Heidelberg, 74, 97-104,2002
[12] Contreras, A., Bedolla, E. , Perez, R., "Interfacial phenomena in wettability of TiC by Al-Mg alloys", Acta Materialia ,52 985-994,2004
[13] Vaucher, S., Beffort, O., "Bonding and interface formation in Metal Matrix Composites", Vol. 9, EMPA Swiss Federal Laboratories for Materials Testing and Research Thun Switzerland,2000
[14] Tham, L.M., Gupta, M. and Cheng, L., "Effect Of Limited Matrix-Reinforcement Interfacial Reaction On Enhancing The Mechanical Properties Of Aluminium-Silicon Carbide Composites", Acta mate., 49 3243-3253,2001
[15] Kevorkijan, V.M. , Sustarsic, B., "A New Production Technology for Discontinuously Reinforced Al-SiC Composites", Key Engineering Materials (Volumes 127 - 131),471-478,1997
[16] Naher, S., Brabazon D., Looney L., "Simulation of The Stir Casting Process, Journal of Materials Processing Technology", 143-144 ,567-571,2003
[17] Yarandi, F.M. , Rohatgi, P.K. , Ray, S., Settling, "Casting Fluidity and Solidification Behavior of Aluminum-SiC Particle Composite", Journal Key Engineering Materials (Volumes 79 - 80), 91-104,1993
[18] J. Hashim, L. Looney* and M. S. J. Hashmi, Metal matrix composites: production by the stir casting method", Journal of Materials Processing Technology,Volumes 92-93, Pages 1-7,1999
[19] Balasivanandha S. P.,, Karunamoorthy, L., Kathiresan, S., Mohan, B., "Influence of stirring speed and stirring time on distribution of particles in cast metal matrix composite", Journal of Materials Processing Technology,Volume 171, Issue 2, , Pages 268-273,2006
[20] A. Ourdjini, K.C. Chew, B.T. Khoo, "Settling of silicon carbide particles in cast metal matrix composite", J. Mater. Process. Technol. 116,72-76.,2001
[21] Aklaghi, F., Lajevardi, A., Maghanaki, H.M., "Effect of Casting Temperature On The Microstructure And Wear Resistance of Compocast A356/SiCp Composites:A Comparison Between SS and SL Routes", J. Mat. Proc. Tech,2004
[22] Hallen, J.M. , Balmori, H.M. , Jaramillo-Vigueras, D. , Estrada, J.L., González J.L. , Manzano-Ramírez, A., "Influence of Mg and Stirring on the Strength of an Aluminium Matrix Composite Obtained by Compocasting", Journal Key Engineering Materials (Volumes 127 - 131), 495-502,1997
[23] Wang,H., 2007, In-Situ Si/Al "Composite Produced by Semisolid Metal Processing, Materials and Manufacturing Processes", 22, 696 - 699,2007
[24] Qin, Q.D., Zhao, , Y.G., Cong, P.J. W. Zhou and Xu, B., "Semisolid microstructure of Mg2Si/Al composite by cooling slope cast and its evolution during partial remelting process", Materials Science and Engineering: A, 444, 99-103,2007
[25] Ghomashchi,M.R.,Vikhrov,A.,"Squeeze casting: an overview",J. of Materials Processing Technology 101,1-9,2000
[26] Vijayaram, T.R., Sulaiman, S., Hamouda, A.M.S. and Ahmad, M.H.M., "Fabrication of fiber reinforced metal matrix composites by squeeze casting technology". Journal of Materials Processing Technology,178,34-38,2006
[27] Yong, M. S. and Clegg, A. J., "Process optimization for a squeeze cast magnesium alloy", J. of Mat. Proc. Tech., 145, 134-141,2004
[28] Zheng,M., Wu, K., Yao, C., "Characterization of interfacial reaction in squeeze cast SiCw/Mg composites", Materials Letters,47, 118-124,2001
[29] Reihani, S.M.S., "Processing of squeeze cast Al6061-30vol% SiC composites and their characterization". Materials and Design,27, 216-222,2006
[30] Long, S., Beffort, O., Cayron, C., Bonjour C., "Microstructure and mechanical properties of a high volume fraction SiC particle reinforced AlCu4MgAg squeeze casting", Mat. Sci. and Eng. A269 175-185,1999
[31] Vicens,J., Chédru, M., Chermant, J. L., "New Al-AlN composites fabricated by squeeze casting: interfacial phenomena", Composites Part A: Applied Science and Manufacturing, Volume 33,Issue10,2, Pages 1421-1423,2002
[32] Spencer, K., Corbin, S.F., Lloyd, D.J., "The Influence of Iron Content on the Plane Strain Fracture Behaviour of AA 5754 Al-Mg Sheet Alloys", Materials Science and Engineering A325,394-404,2002
[33] Valdez,S., Campillo,B., Pérez,R., Martínez,L., García H. A., "Synthesis and microstructural characterization of Al-Mg alloy-SiC particle composite", Materials Letters, 62, 2623-2625,2008
[34] Ürkmez, N., "AlMg3/SiCp Kompozitlerinin Üretimi ve Mekanik Özelliklerdeki İncelenmesi", Doktora Tezi, YTU F.B.E., İstanbul, 2004
[35] Skolianos,S.M., Skolianos, S.M., Kiourtsidis, G. and Xatzifotiou, T. "Effect of Applied Pressure on the Microstructure and Mechanical Properties of Squeeze-Cast aluminium AA6061 alloy",Material Sci. and Engineering A231,17-24,1997

Various methods are used during the production of Metal Matrix Composites (MMC), depending on the type of reinforcement and its geometry. [1]. These methods are liquid, solid and double phase methods. [2-4]. Each method has its own advantages and disadvantages during its application [1,5-7].

Quite a high amount of resistance, homogenous reinforcement distribution, and controlled inter surface reactions can be provided as a result of solid phase production methods in especially particle reinforced metal matrix composite (PRMMC) materials. However the procedure is difficult and quite costly due to additional processes. The particle sizes that can be obtained are limited.[1]

As liquid phase production methods are relatively cheaper, easier and more adaptable they are commercially preferred. During the production of PRMMC materials with liquid phase methods, problems that are difficult to overcome occur at the stirring and solidification processes[4, 8-10]. Some of the main problems that can occur are, not being able to homogenously distribute the reinforcement material into the liquid phase, not being wetted by the matrix material, being pushed beyond the mixture, flocculation, accumulation, occurrence of unwanted chemical reactions between the matrix and reinforcement material, inter surface problems and formation of pores [11-14].

There are several studies that research for solutions of the present problems in literature. Reinforcement pre processes and metallurgical procedures that increase wetting are carried out in order to improve the inter surface connection between the reinforcement and the matrix[15].

Different stirring profiles, stirring speed and durations have been tried in order to overcome problems such as the reinforcement being pushed out of the mixture, flocculation and sedimentation [19,20]. Although these solutions provide homogenous reinforcement, unwanted inter surface reactions are also faced as stirring duration is extended in high temperatures and the rate of pore formation is also increased. [2, 12, 15-20].

The methods using double phase for production are being preferred by investigators recently. These methods have several advantages that can be explained with the ticsotropic behavior of metal materials. Main advantages of said method can be listed as: (a) Lower energy consumption relative to other liquid stirring methods due to short time stirring procedures in low temperatures; (b) reducing chemical waste in the reinforcement material from the alloy (c) longer mold life; (d) laminar flow of the viscose semi solid material; (e) lower solidification shrinkage; (f) lower tendency to hot tearing; (g) faster process conversion; (h) less formation of reaction products that reduce the resistance of composite material; (j) reducing abrasion in the stirrers, and reducing the unwanted elements inside the mixture; (k) less porous inner structure as the gas intake rate from the environment is reduced; (I) solid phase formation having co axial particles which are not dentritic [21-22]. The main disadvantages of the semi solid production methods are; stirring difficulty due to high viscosity and trying to ensure that the procedure parameters are kept fixed (temperature, shear stresses etc.) [21-24].

A method and device for the method of particle reinforced composite metal stirring developed according to the present invention can overcome the disadvantages mentioned above and the characteristics of the method and device developed according to the present invention is as follows:
- Ceramic particles with different ratios are added directly into metal matrix material using the semi solid stirring method,
- Ceramic particles are homogenously distributed into metal or metal alloys which are semi solid,
- The stirring procedure is carried out by means of stirrers having different profiles, prepared from graphite rods when the material is at a semi solid state,
- When the stirring procedure is completed the semi solid mixture is transferred into molds either at a semi solid state or under high temperatures,
- Particle reinforced composite metal production can be performed using the desired casting or production method,
- The product sizes are determined by the mold section and the volume of the crucible; and as a result the particle reinforced composite metal production having the desired characteristics can be carried out.

### Description of the Drawings

The figures that have been drawn in order to further explain the method and device for the production of continuous composite metal foam and particle reinforced composite metal stirring method have been attached to this document. The definitions of the figures are given below.
Figure 1 Process line sectional view
Figure 2 Process line mold movement view
Figure 3 The view of the crucible and the crucible bottom
Figure 4 Schematic view of the furnace
Figure 5 The schematic view of the kneading and stirring apparatus and the stirring system
Figure 6 Schematic view of the bottom of the crucible
Figure 7 View of the aluminum composite foam that has been prepared by adding %25 SiCp reinforcement
Figure 8 SiC reinforcement rate-linear expansion change graphic
Figure 9 View of the non reinforced, %10 SiC reinforced and %20 SiC reinforced samples that have been produced with 5754 alloy
Figure 10 View of the aluminum foam samples that have been produced using TiH₂ powders having different particle sizes,
Figure 11 View of %1 TiH2 and %20 SiC reinforced 5754 alloy that has been foamed at different durations
Figure 12 Resistance graphic according to heat treatment application of composite foam produced with 7075 Aluminum alloy
Figure 13 Resistance graphic of 15% SiC reinforced composite foam not treated with heat and resistance graphic of 20% SiC reinforced composite foam treated with heat Figure 14 Resistance graphics of 15% SiC reinforced composite foam treated with heat
Figure 15 Resistance graphics of composite foam with variable densities but whose aluminum 5754 aluminum materials and reinforcement rates are the same
Figure 16 Resistance graphics of composite foam whose 5083 aluminum materials and reinforcement rates are the same but whose densities are variable
Figure 17 Resistance graphics of composite foam whose 7075 aluminum materials and reinforcement rates are the same but whose densities are variable
Figure 18 Surface images that have been obtained as a result of SEM examinations
Figure 19 Micro rigidity test results of naturally aged and heat treated composite foam samples
Figure 20 View of the characteristic curves of furnace sections
Figure 21 The inner structure sectional view of the composite foam obtained as a result of a graphite mold foaming procedure
Figure 22 The inner structure sectional view of the composite foam obtained as a result of a gas concrete foaming procedure.
Figure 23 The inner structure sectional view of the composite foam produced in a continuous form foam production device

### Descriptions of the parts shown in the figures

The components (parts, elements) within the drawings (figures) that have been prepared in order to further describe the method and device developed by means of the invention for continuous composite metal foam production and particle reinforced composite metal stirring have each been numbered. The descriptions of each number have been listed below.
1 Front heating section
2 Stirring section
3 Foaming section
4 Mold entrance cover
5 Mold exit cover
6 Top stirring cover
7 Resistance groups
8 Moving molds (Material resistant to high temperatures and having low heat transfer)
9 Mold bed
11 Crucible
12 Crucible bottom (Material resistant to high temperatures and having low heat transfer)
13 Reinforcement powder oxidization vessel
14 Protective gas inlet (N₂ or argon)
15 Pushrod
16 Fan
17 Piston
18 Kneading and stirring apparatus
19 Heat sensor
20 Pressure sensor
21 Foaming powder vessel (TiH₂ or CaCO₃)
22 Foaming powder inlet.
23 Matrix material inlet (Particle or powder form)
24 Matrix material vessel
25 Reinforcement powder inlet (SiC, TiC,B₄C or Al₂O₃)
26 Reinforcement powder vessel
27 Stirring mechanism
27a Stirring mechanism rotating means
27b Up and down movement of stirring mechanism means

### Detailed description of the Invention

The present invention is a new method and device used in composite metal foam production; wherein the developed device comprises the following characteristics.

The device that has been developed in order to produce metal foam comprises three sections which are the front heating section (1), the stirring section (2) and the foaming section (3). All sections are heated with separate resistance groups (7). The temperature control of the sections is carried out separately.

The temperatures of the furnace front heating (1) section are temperatures that are below 40 - 60 °C, of the molting temperatures of the metal or metal alloy that is to be foamed.

The temperatures of the foaming section (3) are temperatures that are 50 - 70 °C higher than the molten temperature of the metal or metal alloy that is to be foamed.

The temperatures of the stirring section (2) are 100 - 300 °C higher than the molten temperatures of the metal or metal alloy that is to be foamed.

The movable molds (8) and the reinforcement powders at the front heating section are tried to be brought to process temperatures.

The stirring section (2) comprises a crucible (11), metal or metal alloy material inlet (23) that is to be foamed, reinforcement powder inlet (25), foaming powder inlet (22), protective gas inlet (14) and top stirring cover (6), kneading and stirring apparatus (18) and a stirring mechanism (27). Protective gas (N₂ or argon) is continuously sprayed on a crucible (11).

Reinforcement material, foaming metal or metal alloy (matrix material), foaming powder and powder inputs (25,23,22,and 14) are poured through the inlets located on said stirring section (2).

Protective gas (N₂ or argon) are present all the time in the environment and the protective gas is continuously sprayed on the crucible (11). The reinforcement and matrix material and foaming powder inputs (25,23 and 22) are provided by the automatic control unit according to the information obtained from the sensors (19 and 20). The material inside the metal or metal alloy (matrix material) vessel (24) that is to be foamed, is divided into parts. Said material, can be processed by preparing it in particle or powder form from metal plate, ingot or recycled materials. The materials can be formed of aluminum, copper, titanium, nickel or other metals.

The stirring process with kneading and stirring apparatus (18) is again carried out through the top stirring cover located at again the top alignment of the crucible. Moreover the gas used as protective atmosphere (N₂ or argon) is also blown onto the crucible from this cover section.

The kneading and mixing apparatus (18) are operated by the kneading and stirring mechanism (27). The pressure sensor (20) and the temperature sensor can be located within the stirring mechanism (27). Besides this the temperature sensor (19) can also be located in the crucible (19). The stirring procedures are carried out by controlling the viscosity/consistency and temperature information obtained from the pressure and temperature sensors (19 and 20). One of the most important aspects of the invention is to keep the mixture at a semi solid state during the whole of the stirring process. If the viscosity is low (at the phase of being semi solid to being liquid) the viscosity is increased by adding foaming metal or metal alloy to the mixture. If the viscosity is high (at the phase from being semi solid to solid) the stirring procedure is continued without adding metal to the mixture. The mixture is checked to see if it is at a semi solid state by means of the pressure and temperature sensors (19 and 20) which are controlled by the control unit and the addition of metal is provided by commands submitted to the stirrer by the control unit.

The pressure sensor (20) of the stirring mechanism (27), submits the pressure (viscosity) information that enables to control the up and down movement of the stirrer at the pressure value, to the automatic control unit.

The temperature sensor (19) which measures the temperature inside the crucible (11) submits the temperature information which enables the movement of the stirrer by ensuring that the mixture is kept at a certain temperature, to the automatic control unit.

The stirring mechanism (27) is a system that can operate in connection with a tool changer such that it can provide the changing of different stirrers and that can ensure that the required stirrer at the stirring section is chosen and attached. After the stirrer is attached the down and up (27b) and rotational (27a) movement is carried out. The stirring durations, the selection of stirrers, their attachment or dismantling is controlled by an electronic system.

The end parts of the kneading and stirring apparatus (18) connected to the stirring mechanism (27) can be flat, spiral or could have holes inside it. The holes within the kneading and stirring apparatus with holes, can be circular, elliptical, or can have a square shapes or a polygonal geometrical shapes, and the holes could each be the same size or could be in different sizes.

The kneading and stirring apparatus (18) can be resistant to high temperatures and can have different diameters depending on the crucible diameter. In the case that the bottom of the crucible has a different geometry, the kneading and stirring apparatus (18) can also have different geometries and sizes compliant to the geometry of the crucible.

The material of the stirrers (18) can be made of graphite or said stirrers could be coated with high temperature resistant materials such as ceramic. Besides this, the surface of the apparatus (18) can be coated with a mixture comprising silicium carbide powder and colloidal silica. By this means, the life span of the stirrer is also extended.

More than one crucible (11) can be used which can be moved in sequence in order to provide a mixture that is continuously at a semi solid state. The crucible (11) which is empty is pushed outside of the stirring section (2) by moving it forward and a new crucible (11) is pushed in place to replace the preceding crucible. The next crucible with a mixture prepared inside is brought to an alignment with the movable crucibles and this procedure is repeated constantly to provide a ready mixed mixture.

The bottom parts of the crucibles (11) are open and the front part of the movable mold also functions as a crucible bottom (25) and is at a closed position during the stirring procedures. The movable molds move along the mold bearing (9) made of firebrick that extends from the cover (4) of the movable mold to the mold outlet cover.

The material of the crucible (11) can be SiC, Al₂O₃, graphite etc. The crucible bottom (12) is made of high temperature resistant and heat conducting material. Preferably graphite is used to form crucible bottoms (12). The vessel (13) is made of high temperature resistant and low heat conductive material such as gas, concrete, ceramic foam etc.

A fan (16) mechanism is present on the mold outlet cover so that the foam material exiting out of the furnace can be cooled.

The continuous metal foam production or particle reinforced composite metal production method developed according to the present invention, has been listed below:
1- The movable molds (8) and reinforcement powders at the front part of the furnace (1) is subjected to pre-heating and are brought to process temperatures. Reinforcement powders can be SiC, B₄C, Al₂O₃, TiC, and other carbides, oxides, nitrides and ceramic powders.
2- The pre heating section (1) of the furnace is brought to a temperature approximately below 40-60 °C of the metal or metal alloy melting temperature which is to be turned into foam. The temperature of the foaming section (3) is brought to a temperature 50 - 70 °C higher than the melting temperature of the metal or metal alloy that is to be foamed.
3- The crucible (11) containing metal or metal alloy that is to be turned into foam, is taken into the stirring section (2) of the pre-heating section (1) of the furnace. The temperature of the stirring section (2) is 100 - 300 °C higher than the metal or metal alloy melting temperature that is to be turned into foam.
4- The metal or metal alloy (matrix material) present inside the stirring section (2) of the crucible (11) is kept until the temperature of said mixture rises to the temperature range in which said mixture is at a semi solid state.
5- The movable molds (8) are inserted into the pre-heating section (1) from the mold entry cover (4) and is brought to the temperature of the pre-heating section (1)
6- When the material inside the crucible (11) is softened and begins to be crushed, the reinforcement material that has been pre-heated, is added into the crucible (11) through the reinforcement material inlet (25).
7- The metal or metal alloy (matrix material) that is to be turned into foam is poured in from the crucible inlet (11) in order to ensure that the material stays between the semi solid temperature ranges, when the temperature exceeds the semi solid state temperature range. Metal or metal alloy addition, is carried out by the automatic control unit according to the information obtained from the pressure sensors (20). The viscosity of the mixture is controlled by means of adding metal or metal alloy in accordance with the information obtained from the pressure and temperature sensors (19 and 20). At this point the aim is to ensure that the mixture is kept at a semi solid state. The aim or the mixture to be kept at a semi solid state is to ensure that the material does not flocculate or sedimentation is not created when the reinforcement material is added, and to ensure that the reinforcement material is homogenously distributed into the mixture. If the viscosity of the mixture is low (at the phase from being at a semi solid state to being liquid), the viscosity is increased by adding metal or metal alloy that is to be converted into foam in order to keep the mixture at a semi solid state. If the viscosity of the mixture is high (at the phase from being at a semi solid state to becoming solid) the stirring procedure is continued without adding metal to the mixture. When the temperature of the mixture increases, and when the viscosity is low, reinforcement material is not added to the mixture and only metal or metal alloy is added.
8- The mixture is checked if it is at a semi solid state or not by determining by means of the pressure and temperature sensors (19 and 20) controlled by the control unit, and again the semi solid state is ensured by the commands submitted to the stirrer and metal addition mechanism.
9- After the reinforcement material is added, kneading and mixing procedures are carried out together until the material is homogenously mixed. The stirring process is carried out by the up and down movement of the stirrer(s) depending on the viscosity/stability (or in other words depending on the mixture being at a semi solid state or not) of the material found inside the crucible (11). Besides this the stirrer(s) (18) also change orbits by zig zag or elliptical or radial movement inside the crucible (11).
10- After the mixture is prepared at the desired amount, the foaming powder inside (TiH₂ and CaCO₃ and compounds comprising gas) the foaming powder vessel (21) is added to the mixture through the foaming powder inlet (22) and the quick stirring procedure is repeated. At this moment metal or alloy is continued to be added to the mixture.
11- After the mixture is prepared at the desired amounts, the foaming powder inside the foaming powder vessel (21) is added to the mixture from the foaming powder inlet (22) and the quick stirring process is continued. During this time metal or alloy is continued to be added to the mixture.
12- When a homogenous mixture is obtained, the movable mold is shifted and the bottom of the crucible (11) is opened, the mixture is transferred into the mold cavity (8) from the bottom of the crucible (11) by means of a thrusting piston (17).
13- Whilst the mixture is being pushed by the piston (17) the movable mold is moved at a constant speed on the mold bed (9) by means of a pushrod (15) and the mixture fills the cavity of the movable mold.
14- The movable mold (8) is taken into the foaming section (3) having a temperature which is 50 - 70 °C higher than the melting temperature of the metal or metal alloy that is to be foamed.
15- When the waiting period depending on the mixture amount, is completed the mold (8) is taken out of the furnace by means of the pushrod (15), after the mold exit cover (5) is opened.
16- The foaming material inside the mold which has been taken out of the furnace is cooled quickly by means of cooling fans (16).

### TESTS CARRIED OUT FOR THE PRODUCTION METHOD DEVELOPED ACCORDING TO THE INVENTION

Several tests have been carried out regarding the continuous composite metal foam production developed according to the invention or method developed for the production of metal foam using the particle reinforced metal production method and device developed for the continuous production of metal foam. The tests that have been conducted for the product that was produced using the method subject to the invention have been listed below.
1- Determining the reinforcement powder ratios that could be added into the semi solid material. (Up to 25% reinforcement powder can be added into semi solid material) (Figure 7).
2- Determining the effect of the foaming powder amount to linear expansion (The linear expansion rate is 5-8 when the foaming powder is added at a percentage of 1-2%) (Figure 8)
3- Examining the effect of the reinforcement rate to the formation of foam. The effects of SiC powders to the formation of foam have been mentioned below. When the SiC reinforcement amount increased;
- Linear expansion increased
- Homogenous pore distribution was provided
- Drainage formation was prevented
- The thickness of the cell walls increased
- The resistance of the cell walls increased and pore combining was prevented
The effects mentioned above are performed by the selection of the foam formation temperature distinctive to the material. When the waiting period at a high temperature has been exceeded, combining of the pores, thinning of the cell walls and sedimentation occurs.
4- Examining the effect of the foaming powder size to the formation of foam. (when foaming powder having particle sizes larger than ∼40 µm was used it was harder for a homogenous inner structure to be obtained. The test results are shown in Figure 10).
5- Examining the effect of the type of foaming powder used to the production of foam. Similar results have been obtained with tests carried out with TiH₂ and CaCO₃ powders. The process parameters change for such procedures.
6- Examining the effect of the foaming duration to the foam structure. As the duration for the foaming procedure increased the cell sizes increased, and the cells are combined with each other and a non homogenous inner structure is obtained. The pore structure in stirring and foaming procedures carried out under protective gas by means of the metal foam production apparatus passes through different phases depending on time. The time also changes depending on material. The %1 TiH₂ and %20 SiC reinforced 5754 alloy foam which have been foamed in different durations can be seen in Figure 11.
7- Measuring the densities of the products that have been produced. Aluminum composite foam materials having a density between 0.3 gr/cm³ to 0.8 gr/cm³ have been obtained. The results of the tests carried out in relation to specific weight and relative densities (EN AW 5754) have been given in the table below.

| Test name | Condensation (g/cm3) | Relative densities | Test Name | Condensation (g/cm3) | Relative densities |
|---|---|---|---|---|---|
| **TiH2**1**SiC**2 **TB**44µm**KS** 8min-heat tr | 0,588 | 0,220 | **TiH2**1**SiC**20**TB**30µ**mKS**12min-heat tr | 0,379 | 0,141 |
| **TiH2**1**SiC**20**TB**44µm**KS**10min -heat tr | 0,399 | 0,149 | **TiH2**1 **SiC**10**TB**4µm **KS** 8min | 0,618 | 0,231 |
| **TiH2**1**SiC**20**TB**44µm**KS**12min -heat tr | 0,388 | 0,145 | **TiH2**1**SiC**10**TB**4µm **KS** 10min | 0,652 | 0,244 |
| **TiH2**1**SiC**0**TB**44µm**KS**8min-heat tr | 0,497 | 0,186 | **TiH2**1 **SiC**10**TB**4µm**KS** 12min | 0,550 | 0,205 |
| **TiH2**1**SiC**0**TB**44µm**KS**10min heat tr | 0,497 | 0,186 | **TiH2**1**SiC**10**TB**4µm**KS**8min-heat tr | 0,769 | 0,288 |
| **TiH2**1**SiC**0**TB**44µm**KS1**2min-heat tr | 0,410 | 0,153 | **TiH2**1**SiC**10**TB**4µm**KS**10min heat tr | 0,662 | 0,247 |
| **TiH2**1**SiC**0**TB**44µm**KS** 10min | 0,389 | 0,145 | **TiH2**1 **SiC**10 **TB**4µm**KS** 12min-heat tr | 0,683 | 0,255 |
| **TiH2**1 **SiC2**0**TB**44µm **KS** 8min | 0,324 | 0,121 | **TiH2**1 **SiC** 20 **TB**4µm 8min | 0,613 | 0,229 |
| **TiH2**1 **SiC**20**TB**44µm **KS** 10min | 0,380 | 0,142 | **TiH2**1**SiC**20**TB**4µm**KS** 10min | 0,773 | 0,289 |
| **TiH2**1**SiC2**0**TB**44µm **KS** 12min | 0,311 | 0,116 | **TiH2**1 **SiC** 20**TB**4µm**KS** 12min | 0,960 | 0,359 |
| **TiH2**1**SiC**10**TB**44µm**KS**8min-heat tr. | 0,704 | 0,263 | **TiH2**1**SiC**10**TB**100µm**KS** 8min | 0,648 | 0,242 |
| **TiH2**1**SiC**10**TB**44µm**KS**10min -heat tr. | 0,683 | 0,255 | **TiH2**1**SiC**10**TB**100µm**KS**10mi n | 0,521 | 0,195 |
| **TiH2**1**SiC1**0**TB**44µm**KS**12min -heat tr. | 0,482 | 0,180 | **TiH2**1**SiC**10**TB**100µm**KS** 12min | 0,499 | 0,186 |
| **TiH2**1**SiC**10 **TB**44µm **KS**8min | 0,473 | 0,177 | **TiH2**1**SiC**20**TB**100µm**KS** 8min | 0,334 | 0,125 |
| **TiH2**1 **SiC**10 **TB**44µm **KS**10min | 0,380 | 0,142 | **TiH2**1**SiC**20**TB**100µm **KS**10min | 0,371 | 0,138 |
| **TiH2**1 **SiC**10**TB**44µm **KS** 12min | 0,413 | 0,154 | **TiH2**1**SiC**20**TB**100µm**KS** 12min | 0,450 | 0,168 |
| **TiH2**1**SiC**20**TB**44µm**KS**8min 800°C | 0,900 | 0,337 | **TiH2**1**SiC**10**TB**100µm **KS** 8min-heat tr. | 0,493 | 0,184 |
| **TiH2**1**SiC**20**TB**44µm**KS**10min 800 °C | 0,665 | 0,249 | **TiH2**1**SiC**10**TB**100µm**KS**10mi n-heat tr. | 0,260 | 0,097 |
| **TiH2**1**SiC**20**TB**44µm**KS**12min 800 °C | 0,616 | 0,230 | **TiH2**1**SiC**10**TB**100µm**KS**12mi n-heat tr.- | 0,290 | 0,108 |
| **TiH2**1 **SiC**10**TB**30µm**KS** 8min-heat tr. | 0,564 | 0,211 | **TiH2**1**SiC**20**TB**100µm **KS** 8min-heat tr.- | 0,408 | 0,152 |
| **TiH2**1**SiC**10**TB**30µm**KS**10min -heat tr. | 0,365 | 0,136 | **TiH2**1**SiC**20**TB**100µm**KS**10mi n-heat tr.- | 0,772 | 0,289 |
| **TiH2**1**SiC**10**TB**30µm**KS**12min -heat tr. | 0,418 | 0,156 | **TiH2**1**SiC**20**TB**100µm**KS**12mi n -heat tr. | 0,575 | 0,215 |
| **TiH2**1**SiC** 10 **TB**30µm **KS** 8min | 0,300 | 0,112 | **TiH2**0,5**SiC**20**TB**44µm **KS** 8min | 0,424 | 0,158 |
| **TiH2**1**SiC**10**TB**30µm **KS** 10min | 0,249 | 0,093 | **TiH2**0,5**SiC**20**TB**44µm**KS**10mi n | 0,301 | 0,112 |
| **TiH2**1**SiC**10 **TB**30µm**KS** 12min | 0,346 | 0,129 | **TiH2**0,5**SiC**20**TB**44µm**KS**12mi n | 0,378 | 0,141 |
| **TiH2 SiC** 20 **TB**30µm **KS** 8min | 0,482 | 0,180 | **TiH2SiC**20**TB**44µm **KS** 8min | 0,456 | 0,170 |
| **TiH2**1**SiC** 20**TB**30µm**KS** 10min | 0,590 | 0,22 | **TiH2**2 **SiC**20**TB**44µm **KS**10min | 0,355 | 0,132 |
| **TiH2**1**SiC**20**TB**30µm **KS** 12min | 0,550 | 0,205 | **TiH2**2**SiC**20**TB**44µm**KS** 12min | 0,368 | 0,137 |
| **TiH2**1**SiC**20**TB**30µm**KS** 8min-heat tr. | 0,480 | 0,179 | **TiH2**0,5 **SiC** 5 **TB**44µm **KS**10min | 0,572 | 0,214 |
| **TiH2**1**SiC**20**TB**30µm**KS**10min -heat tr. | 0,643 | 0,240 | **TiH**20,5 **SiC** 10 **TB**44µm **KS**10min | 0,689 | 0,258 |

| | | | | | |
|---|---|---|---|---|---|
| **TiH2**1 **SiC** 20 **TB**30µm **KS(Foaming Time)** 10min-heat tr.-T800 °C → %1 **TiH2**-%20 **SiC-**30µm **P**article **S**ize-10 minutes **Foaming Time- heat tr.** Heat Treatment TiH2 - T800Furnace temperature- All tests besides T800 have been carried out at a furnace temperature of 750 °C). | | | | | |

8- Determining the compressive strengths of the obtained products (Aluminum composite foam materials between the range of 5 MPa- 35 MPa have been produced.
Figure 12, shows that the resistances of the composite foam produced with 7075 aluminum alloy can be increased by means of heat treatment.
Figure 13, shows that the resistance of the composite foam produced using heat treated %20 SiC reinforcement is much higher than non heat treated %15 SiC reinforced composite foam.
Figure 14, shows the effect of the reinforcement rate on resistance. It shows that the composite foam which has been subjected to heat treatment having a higher reinforcement rate is more resistant.
Figure 15, 16 and 17, shows that the resistance of the composite foams with higher density is more resistant in comparison to composite foams having the same material and reinforcement rate but having different densities.
9- The surface images obtained as a result of SEM examinations are shown in Figure 18.
10- The results of the micro rigidity tests have been shown in Figure 19.

### TESTS CARRIED OUT ON THE DEVICE ON WHICH THE PRODUCTION METHOD DEVELOPED ACCORDING TO THE INVENTION IS APPLIED:

The tests related to the device on which the continuous composite metal foam production or particle reinforced composite metal production method developed according to the invention is carried out have been listed below.
1- Forming the temperature characteristic curves of furnace sections: As it can be seen in Figure 20, the furnace sections rise up to 750°C temperature in 3 hours. The characteristics of the device used for measurements are described below.

### Technical features of the AFM05 device

Maximum temperature: 1200 °C
Constant usage temperature: 750 °C
Temperature deviation: + 3 °C
Inner dimensions: 2x (30x30x60) + (40x40x70) (cm)
Heating means: Kanthal (d=2mm) On the ceramic rod, on the side walls of the partitions
Temperature control devices: 3x (PC 442/6, Dual Display,PID.6 step programming)

### Energy distribution

Pre-heating section: 3.85 kW,
Stirring Section: 7.7 kW,
Retention section: 3.85 kW
Total 15.4 kW
Atmosphere: Gas metal protection environment (Nitrogen gas)

2- It has been noted that during the foaming procedures carried out using graphite and gas concrete blocks in tests determining the foam mold materials, low heat conducting material needs to be used as mold material. The inner structure sectional views of the composite foams obtained in tests have been shown in Figures 21 and 22. Heterogeneous pores are present and drainage sections are established inside the inner structure of the composite foam produced in graphite molds. Pores which are homogenous and do not have drainage sections are formed inside the inner structure of the composite foam foamed with gas concrete molds.
The inner structure sectional view of the composite foam in constant from obtained by means of the AFM05 device has been shown in Figure 23. The important issue here is for the composite foam to be produced continuously. The inner structure and density of the foam is controlled by selecting suitable parameters (such as waiting time, TiH₂ size, SiC amount/rate).

The method developed according to the present invention can also be used during the stirring phase of the particle reinforced composite metal production. The steps of the particle reinforced composite metal stirring method have been listed below.
1- The reinforcement powders at the pre heating part of the furnace (1) are subjected to pre-heating and are brought to process temperatures. Reinforcement powders can be SiC, B₄C, Al₂O₃, TiC, and other carbides, oxides, nitrides and ceramic powders.
2- The pre heating section (1) of the furnace is brought to a temperature approximately below 40-60 °C of the metal or metal alloy melting temperature which is to be turned into particle reinforced composite metal.
3- The crucible (11) containing metal or metal alloy that is to be turned into particle reinforced composite metal, is taken into the stirring section (2) of the pre-heating section (1) of the furnace. The temperature of the stirring section (2) is 100 - 300 °C higher than the metal or metal alloy melting temperature that is to be turned into particle reinforced composite metal.
4- The metal or metal alloy used to produce composite metal production inside the crucible (11) located at the stirring section (2) is kept until the temperature thereof is increased to the temperature range wherein said metal or metal alloy is at a semi solid state,
5- When the material inside the crucible (11) is softened and begins to be crushed, the reinforcement material that has been pre-heated, is added into the crucible (11) through the reinforcement material inlet (25).
6- The metal or metal alloy (matrix material) that is to be turned into composite metal production is poured in from the crucible inlet (11) in order to ensure that the material stays between the semi solid temperature range, when the temperature exceeds the semi solid state temperature range. Metal or metal alloy addition, is carried out by the automatic control unit according to the information obtained from the pressure sensors (20). The viscosity of the mixture is controlled by means of adding metal or metal alloy in accordance with the information obtained from the pressure and temperature sensors (19 and 20). At this point the aim is to ensure that the mixture is kept at a semi solid state. The aim or the mixture to be kept at a semi solid state is to ensure that the material does not flocculate or sedimentation is not created when the reinforcement material is added, and to ensure that the reinforcement material is homogenously distributed into the mixture. If the viscosity of the mixture is low (at the phase from being at a semi solid state to being liquid), the viscosity is increased by adding metal or metal alloy that is to be converted into foam in order to keep the mixture at a semi solid state. If the viscosity of the mixture is high (at the phase from being at a semi solid state to becoming solid) the stirring procedure is continued without adding metal to the mixture. When the temperature of the mixture increases, and when the viscosity is low, reinforcement material is not added to the mixture and only metal or metal alloy is added.
7- The mixture is checked if it is at a semi solid state or not by determining by means of the pressure and temperature sensors (19 and 20) controlled by the control unit, and again the semi solid state is ensured by the commands submitted to the stirrer and metal addition mechanism.
8- After the reinforcement material is added, kneading and mixing procedures are carried out together until the material is homogenously mixed. The stirring process is carried out by the up and down movement of the stirrer(s) depending on the viscosity/stability (or in other words depending on the mixture being at a semi solid state or not) of the material found inside the crucible (11). Besides this the stirrer(s) (18) also change orbits by zig zag or elliptical or radial movement inside the crucible (11).
9- When a homogenous mixture is obtained, the composite mixture inside the crucible (11) is taken out and poured into molds thereby a particle reinforced composite material production is obtained by means of a casting or production method.

## Claims

1. A continuous composite metal foam production method, **characterized in that** it comprises the following steps,
• The movable molds (8) and reinforcement powders, are subjected to preheating at the pre heating section (1) of the furnace having a temperature 40 - 60 °C below the melting temperature of the metal or metal alloy that is to be converted into foam,
• The crucible (11) containing metal or metal alloy used to produce foam, is delivered to the stirring section (2) having a temperature 100 - 300 °C higher than the melting temperature of the metal or metal alloy that is to be turned into foamed and the metal or metal alloy to be foamed is added into said crucible,
• Waiting for the temperature of the metal or metal alloy that is to be turned into foam present inside the crucible (11) to increase and reach the temperature range where the metal or metal alloy becomes semi solid,
• Taking the movable molds (8) from the mold inlet cover (4) and moving them to the pre-heating section (1) and bringing the temperature to the pre heating section's (1) temperature,
• When the material inside the crucible (11) is softened and crushed, the reinforced material that has been passed through preheating is added into the crucible (11) via the reinforced material inlet (25),
• In order to ensure that the metal or metal alloy that is to be foamed, inside the crucible (11) is kept at a semi solid temperature range, if the viscosity of the mixture (from being a semi solid to being liquid) is low according to the information obtained from the pressure and temperature sensors (19 and 20) metal or metal alloy to be foamed is added to the mixture in order to increase the viscosity of the mixture, **during this time, no more reinforcement material is added;** and if the viscosity is high the stirring procedure is continued without adding metal or metal alloy to the mixture, thereby keeping the mixture at a semi solid state and continuing this process until the addition of reinforcement material is finished.
• After the mixture is prepared at the desired amount, the foaming powder found inside the foaming powder vessel (21) is added into the mixture through the foaming powder inlet (22) and the stirring procedure is carried out quickly and at this moment, metal or metal alloy is continue to be added into the mixture,
• When a homogenous mixture has been provided, the movable mold is shifted and the bottom of the crucible (11) is opened, and the mixture is pushed by a pushing piston (17) from the bottom of the crucible (11) and transferred to the cavity of the movable mold (8),
• When the mixture is pushed by the piston (17) the mixture is moved at a constant quick speed in the mold bearing (9) by means of a pushrod (15) and the mixture fills the cavity of the movable mold,
• The movable mold (8) is taken into the foaming section (3) having a temperature 50 - 70 °C higher than the melting temperature of the metal or metal alloy that is to be foamed,
• When the waiting time depending on the amount of the mixture is fulfilled the pushrod (15) pushes the outlet cover (5) of the mold (8) and the mixture is taken out of the furnace,
• The foam material inside the mold is quickly cooled by means of cooling fans (16).

2. A particle reinforced composite metal stirring method; **characterized in that**;
• The reinforcement powders are pre heated at the pre heating (1) section and are brought to process temperatures,
• The pre heating section (1) of the furnace is brought to a temperature 40 - 60 °C below the melting temperature of the metal or metal alloy that is to be turned into particle reinforced composite metal,
• The crucible (11) containing metal or metal alloy used to produce particle reinforced composite metal production is taken to the stirring section (2) of the furnace and the temperature of the stirring section (2) is 100 - 300 °C higher than the melting temperature of the metal or metal alloy used to produce composite metal production,
• The metal or metal alloy used to produce composite metal production inside the crucible (11) located at the stirring section (2) is kept until the temperature thereof is increased to the temperature range wherein said metal or metal alloy is at a semi solid state,
• When the material inside the crucible (11) is softened and crushed, the reinforced material that has been passed through preheating is added into the crucible (11) via the reinforced material inlet (25),
• In order to ensure that the material, inside the crucible is kept at a semi solid temperature range, when the temperature exceeds the semi solid temperature, the metal or metal alloy that is used to produce composite metal is added to the crucible (11) or the addition of the metal or metal alloy, is performed by an automatic control unit according to the information obtained from the pressure sensors (20), the viscosity of the mixture is controlled by adding metal or metal alloy according to the information obtained from the pressure and temperature sensors (19 and 20), in order to keep the mixture at a semi solid state, if the viscosity of the mixture is low metal or metal alloy used to produce composite metal is added to the mixture in order to increase the viscosity of the mixture, and if the viscosity of the mixture is high the stirring procedure is continued without adding metal to the mixture, and if the temperature of the mixture increases but the viscosity decreases, reinforcement material is not added to the mixture but only metal or metal alloy is added.
• The mixture is checked if it is at a semi solid state or not by determining by means of the pressure and temperature sensors (19 and 20) controlled by the control unit, and again the semi solid state is ensured by the commands submitted to the stirrer and metal addition mechanism.
• After reinforcement material is added the stirring procedure is carried out by moving the stirrers up and down and at the same time the stirrers move inside the crucible (11) radially or elliptically or in zig zag shape by changing place on the orbit in order to carry out the kneading and stirring procedure together until the material is homogenously mixed by means of stirrers following the addition of reinforcement material,
• When a homogenous mixture is obtained, the composite mixture inside the crucible (11) is taken out and poured into molds thereby a particle reinforced composite material production is obtained by means of a casting or production method.

3. A method according claim 1 and 2 **characterized in that**; the reinforcement material is SiC, B₄C, Al₂O₃, TiC, and other carbides, oxides, nitrides and ceramic.

4. A method according to claims 1 or 2, **characterized in that** the kneading and stirring apparatus (18) which carries out the kneading and stirring procedure at the same time with the homogenously mixing of the material, is moved up and down, and at the same time, radially, elliptically within the crucible (11) or changes place on a zig zag orbit.

5. A continuous composite metal foam production method according to claim 1, **characterized in that** the foaming powder is TiH₂ and CaCO₃.

6. A device for producing composite metal or for performing particle reinforced composite metal stirring, **characterized in that**; it comprises three sections, which are the pre heating section (1), stirring section (2) and foaming section (3), each section (1,2,3) being heated with separate resistance groups (7); wherein temperature controls can be carried out separately; and wherein the temperature of the pre heating (1)section of the furnace is at a temperature lower than 40 - 60 °C, the temperature of the foaming section(3) is at temperature which is higher than 50 - 70 °C of the melting temperature of the metal or metal alloy that is to be foamed, and wherein the temperature of the stirring section (2) is 100 - 300 °C higher than the melting temperature of the metal or metal alloy that is to be foamed.

7. A device for producing composite metal or for performing particle reinforced composite metal stirring according to claim 6, **characterized in that**; the stirring section (2) comprises a crucible (2), inlet (23) for the metal or metal alloy material that is to be foamed, matrix material vessel (24), reinforcement material inlet (25), foaming powder inlet (22), protective gas inlet (14) and a stirring mechanism (27) together with a top stirring cover (6), kneading and stirring apparatus (18); wherein protective gas (N₂ or argon) is continuously sprayed onto the crucible (11).

8. A device for producing composite metal or for performing particle reinforced composite metal stirring according to claim 6 or 7, **characterized in that**; the reinforcement material, matrix material and foaming powder additions (25,23, and 22) are provided by the automatic control unit, according to the information obtained from the sensors (19 and 20).

9. A device for producing composite metal or for performing particle reinforced composite metal stirring according to claim 6 or 7, **characterized in that**; the material inside the metal or metal alloy vessel (24) that is to be foamed or turned into particle reinforced composite, is divided into small pieces.

10. A device for producing composite metal or for performing particle reinforced composite metal stirring according to claim 6 or 7, **characterized in that**; the material inside the metal or metal alloy vessel (24) that is to be foamed or turned into particle reinforced composite is prepared and processed in particle or powder form made from metal plate, ingot or recycled materials.

11. A device for producing composite metal or for performing particle reinforced composite metal stirring according to claim 6 or 7, **characterized in that**; the metal or metal alloy material that is to be foamed or turned into particle reinforced composite, can be comprised of aluminum, copper, titanium, nickel or other metals.

12. A device for producing composite metal or for performing particle reinforced composite metal stirring according to claim 6 or 7, **characterized in that**; the kneading and stirring apparatus (18) are operated by the kneading stirring mechanism (27), the pressure sensors (20) and the temperature sensors (19) are located inside the stirring mechanism (27), that the stirring procedure is carried out by the automatic control unit in a controlled manner according to the viscosity/stability and temperature information obtained from the pressure and temperature sensors (19 and 20).

13. A device for producing composite metal or for performing particle reinforced composite metal stirring according to claim 6 or 7, **characterized in that**; the mixture is kept at a semi solid state during the stirring period, and if the viscosity is low (from being a semi solid to being liquid) the viscosity is increased by adding metal or metal alloy to be foamed, and if the viscosity is high no additional metal is added to the mixture but the stirring process is continued and the pressure and temperature sensors (19 and 20) controlled by the control unit are used to determine if the mixture is at a semi solid state and the stirring process is carried out again by the commands sent to the stirrer and metal addition mechanism by the control unit.

14. A device for producing composite metal or for performing particle reinforced composite metal stirring according to claim 6 or 7, **characterized in that**; the kneading and stirring apparatus (18) connected to the stirring mechanism (27) carries out an up and down (27b) motion and a radial (27a) movement and the stirring times and selection of stirring rods, their attachment and dismantling are controlled by the electronic system.

15. A device for producing composite metal or for performing particle reinforced composite metal stirring according to claim 6 or 7, **characterized in that**; the ends of the kneading and stirring apparatus (18) connected to the stirring mechanism (27) can be flat, spiral or perforated.

16. A device for producing composite metal or for performing particle reinforced composite metal stirring according to claim 6 or 7, **characterized in that**; the holes in the perforated kneading and stirring apparatus (18) ends can have round, square, elliptical, rectangular, or polygonal geometrical shapes and each hole can be of the same size or can be in different sizes.

17. A device for producing composite metal or for performing particle reinforced composite metal stirring according to claim 6 or 7, **characterized in that**; the material of the kneading and stirring apparatus (18) is coated with high temperature resistant material such as graphite or ceramic.

18. A device for producing composite metal or for performing particle reinforced composite metal stirring according to claim 6 or 7, **characterized in that**; the surface of the kneading and stirring apparatus (18) is coated with a mixture prepared from silicium, carbide powder and colloidal silica.

19. A device for producing composite metal or for performing particle reinforced composite metal stirring according to claim 6 or 7, **characterized in that** it comprises a plurality of crucibles (11) which can be moved such that they can be used in sequence in order to provide a semi solid ready mixture constantly, that the empty crucible (11) is pushed forward out of the stirring section (2), a new crucible (11) is pushed in place, the next crucible loaded with the mixture is pushed into queue to be aligned with the molds and that this procedure is repeated to provide ready mixtures continuously.

20. A device for producing composite metal or for performing particle reinforced composite metal stirring according to claim 6 or 7, **characterized in that**; the bottom parts of the crucibles (11) are open, that the front section of the movable mold also functions as the crucible bottom (25), and that said bottom part is at a closed position during the stirring processes.

21. A device for producing composite metal or for performing particle reinforced composite metal stirring according to claim 6 or 7, **characterized in that**; the movable molds are moved on a mold bed (9) made of firebricks that extend from the inlet cover (4) of the mold to the outlet cover of the mold.

22. A device to produce composite metal foam and for stirring particle reinforced composite metal according to claim 6 or 7, **characterized in that** the crucible (11) material is SiC, Al₂O₃ or graphite.

23. A device to produce composite metal foam and for stirring particle reinforced composite metal according to claim 6 or 7, **characterized in that** the bottom of the crucible (12) is made of high temperature resistant and high heat conductive material, preferably graphite.

24. A device to produce composite metal foam and for stirring particle reinforced composite metal according to claim 6 or 7, **characterized in that** the vessel (13) is made of high temperature resistant and low heat conductive material.

25. A device to produce composite metal foam and for stirring particle reinforced composite metal according to claim 6 and 7, **characterized in that** the vessel (13) is gas concrete or ceramic foam.

26. A device to produce composite metal foam or for stirring particle reinforced composite metal according to claim 6, **characterized in that**, a fan (16) mechanism is present on the mold exit cover so that the foam material taken out of the furnace can be cooled down.

## Patentansprüche

1. Eine kontinuierliche Verbundmetallschaumproduktionsmethode, **dadurch gekennzeichnet, daß** sie folgende Schritte beinhaltet,
• Die bewegbaren Gussformen (8) und Verstärkungspulver sind unterworfen zur Vorwärmung an Vorwärmestation (1) des Schmelzofens mit einer Temperatur 40 - 60°C unter der Schmelztemperatur des Metalls oder Metalllegierung, die in Schaum verwandelt werden soll,
• Der Schmelztiegel (11), der das Metall oder die Metalllegierung, die für Schaumproduktion verwendet wird, beinhaltet, ist angeliefert zur Rührstation (2) mit einer Temperatur 100 - 300°C höher als der Schmelztemperatur des Metalls oder Metall-legierung, die in Schaum umgewandelt wird und das geschäumte Metall oder die Metalllegierung ist hinzugefügt in den besagten Schmelztiegel,
• Warten für die Temperatur des Metalls oder der Metalllegierung, die in Schaum verwandelt werden soll, der im Schmelztiegel (11) vorhanden ist, um den Temperaturbereich zu erhöhen und erreichen, wo das Metall oder die Metalllegierung halbfest wird,
• Nehmen der bewegbaren Gussformen (8) vom Gusseinlassdeckel (4) und deren Transport in die Vorwärmestation (1) und Anbringen der Temperatur zu jener Temperatur der Vorwärmestation (1),
• Wenn das Material im Schmelztiegel (11) erweicht und zerbrochen wird, wird das Verstärkungsmaterial, das zur Vorwärmung durchgelaufen ist, in den Schmelztiegel (11) hinzugefügt durch den Verstärkungsmaterialeinlass (25),
• Um sicherzustellen, daß das Metall oder die Metalllegierung, die geschäumt ist, im Schmelztiegel (11) an einem halbfesten Temperaturbereich gehalten werden, falls die Viskosität der Mischung (vom einem halbfesten Aggregatszustand zum flüssigen Zustand) niedrig ist nach der Information erhalten vom Druck- und Temperatursensoren (19 und 20) Metall oder Metalllegierung, die geschäumt ist, ist hinzugefügt in die Mischung, um deren Viskosität zu erhöhen, **im Verlauf dieser Zeit, keine weitere Verstärkungsmaterial ist hinzugefügt;** und falls die Viskosität hoch ist, der Einmischungsprozedur ist weitergeführt ohne Zugabe von Metall oder Metalllegierung, dadurch Einhaltung der Mischung an einem halbfesten Aggregatszustand und Weiterführung dieses Prozesses bis die Zugabe des Verstärkungsmaterials beendet ist.
• Nachdem die Mischung in gewünschter Menge vorbereitet ist, das Schaumpulver befunden im Schaumpulverbehälter (21) ist hinzugefügt in die Mischung durch den Schaumpulvereinlass (22) und Einmischungsprozedur schnell und exakt an diesem Moment durchgeführt wird, wird weiter das Metall oder die Metalllegierung in die Mischung hinzugefügt,
• Wenn eine homogene Mischung sichergestellt wird, wird die bewegbare Gussform verschoben und der Boden des Schmelztiegels (11) ist geöffnet, und die Mischung ist verschoben mit einem Schiebekolben (17) vom Boden des Schmelztiegels (11) und übertragen zum Hohlraum der bewegbaren Gussform (8),
• Wenn die Mischung vom Kolben (17) verschoben wird, wird die Mischung an einer konstanten Schnellgeschwindigkeit in das Gusslager (9) geschoben durch einen Schiebearm (15) und die Mischung füllt den Hohlraum der bewegbaren Gussform ein,
• Die bewegbare Gussform (8) ist aufgenommen in die Schaumstation (3) mit einer Temperatur 50 - 70°C höher als der Schmelztemperatur des Metalls oder der Metalllegierung, die geschäumt wird,
• Wenn die Wartezeit in Abhängigkeit von der Menge der Mischung eingefüllt ist, schiebt der Schiebearm (15) den Ausflussdeckel (5) der Gussform (8) und die Mischung ist herausgenommen aus dem Schmelzofen,
• Schaummaterial in der Gussform ist schnell abgekühlt durch die Kühlerlüfter (16).

2. Eine durch Partikeln verstärkte Verbundmetalleinmischungsmethode; **dadurch gekennzeichnet, daß**
• Verstärkungspulver an Vorwärmestation (1) erwärmt und zur Prozesstemperaturen hingebracht werden,
• Die Vorwärmestation (1) des Schmelzofens ist aufgebracht zu einer Temperatur 40 - 60°C unter der Schmelztemperatur des Metalls oder der Metalllegierung, die umgewandelt wird in durch Partikeln verstärkte Verbundmetall,
• Der Schmelztiegel (11), der das Metall oder die Metalllegierung, die für durch Partikeln verstärkte Verbundmetallproduktion verwendet wird, ist die Produktion angeliefert zur Rührstation (2) des Schmelzofens und die Temperatur der Rührstation (2) ist 100 - 300°C höher als der Schmelztemperatur des Metalls oder der Metalllegierung, die verwendet wird für die Produktion von Verbundmetall,
• Das Metall oder die Metalllegierung, die für die Produktion von Verbundmetall im Schmelztiegel (11) verwendet wird, der an Rührstation (2) gehalten wird, bis deren Temperatur erhöht ist zum Temperaturbereich, wo besagte Metall oder Metalllegierung an einem halbfesten Aggregatszustand ist,
• Wenn das Material im Schmelztiegel (11) erweicht und zerbrochen wird, wird das Verstärkungsmaterial, das zur Vorwärmung durchgelaufen ist, in den Schmelztiegel (11) hinzugefügt durch den Verstärkungsmaterialeinlass (25),
• Um sicherzustellen, daß das Material im Schmelztiegel an einem halbfesten Temperaturbereich gehalten wird, wird das Metall oder die Metalllegierung, die für Verbundmetallproduktion verwendet wird, ist hinzugefügt in den Schmelztiegel (11) oder die Hinzufügung vom Metall oder von der Metalllegierung ist durchgeführt von einer automatischen Kontrolleinheit nach der Information erhalten von Drucksensoren (20), die Viskosität der Mischung ist kontrolliert durch Zugabe von Metall oder Metalllegierung nach der Information erhalten von Druck- und Temperatursensoren (19 und 20), um die Mischung an einem halbfesten Aggregatszustand zu halten, falls die Viskosität der Mischung niedrig ist, wird das Metall oder die Metalllegierung, die für Verbundmetallproduktion verwendet wird, ist hinzugefügt in die Mischung, um die Viskosität der Mischung zu erhöhen, und falls die Viskosität der Mischung hoch ist, wird der Einmischungsprozedur weitergeführt ohne ein Metall in die Mischung zuzugeben, und falls die Temperatur der Mischung sich erhöht, aber die Viskosität sich erniedrigt, Verstärkungsmaterial ist nicht hinzugefügt in die Mischung, aber nur Metall oder Metalllegierung wird zugegeben.
• Die Mischung wird geprüft, ob sie an einem halbfesten Aggregatszustand ist oder nicht durch Feststellung von Druck- und Temperatursensoren (19 und 20), die von Kontrolleinheit kontrolliert werden, und wiederum wird der halbfeste Aggregatszustand sichergestellt von Befehle eingegeben zum Rührer- und Metallhinzufügungs-mechanismus.
• Nach der Zugabe von Verstärkungsmaterial der Einmischungsprozedur ist durchgeführt durch die Bewegung der Rührer auf und ab und in der selben Zeit bewegen sich die Rührer in den Schmelztiegel (11) radial oder elliptisch oder in zig zag Form durch Veränderung des Platzes auf dem Orbit, um den Kneten- und Einmischungsprozedur zusammen durchzuführen, bis das Material homogen eingemischt wird mit Rührer nach der Zugabe von Verstärkungsmaterial,
• Wenn eine homogene Mischung erhalten wird, wird die zusammengesetzte Mischung im Schmelztiegel (11) herausgenommen und in Gussformen eingegossen, damit wird ein durch Partikel verstärkte Verbundmaterialproduktion erhalten durch eine Gieß- oder Produktionsmethode.

3. Eine Methode nach den Ansprüche 1 und 2, **dadurch gekennzeichnet, daß** das Verstärkungsmaterial SiC, B₄C, Al₂O₃, TiC, und andere Karbide, Oxide, Nitride und Keramik ist.

4. Eine Methode nach den Ansprüche 1 oder 2, **dadurch gekennzeichnet, daß** der Kneten- und Einmischungsapparat (18), die den Kneten- und Einmischungsprozedur durchführt in der selben Zeit mit der homogene Einmischung des Materials, auf und ab bewegt, und in der selben Zeit, radial, elliptisch im Schmelztiegel (11) oder den Platz verändert auf einem zig zag Orbit.

5. Eine kontinuierliche Verbundmetallschaumproduktionsmethode nach Anspruch 1, **dadurch gekennzeichnet, daß** Schaumpulver TiH₂ und CaCO₃ ist.

6. Ein Gerät für die Produktion von Verbundmetall oder für die Ausführung der Rührung vom durch Partikel verstärkte Verbundmetall, **dadurch gekennzeichnet, daß** es drei Stationen besitzt, die Vorwärmestation (1), Rührstation (2) und Schaumstation (3) sind, jede Station (1,2,3) sind erwärmt von einzelnen Widerstandsgruppen (7); wo Temperaturkontrollen getrennt durchgeführt werden können; und wo die Temperatur der Vorwärmestation (1) des Schmelzofens an einer Temperatur ist kleiner als 40 - 60°C, die Temperatur der Schaumstation (3) ist an einer Temperatur, die höher ist als 50 - 70°C der Schmelztemperatur des Metalls oder der Metalllegierung, de geschäumt wird, und wo die Temperatur der Rührstation (2) 100 - 300°C höher ist als der Schmelztemperatur des Metalls oder der Metalllegierung, die geschäumt wird.

7. Ein Gerät für die Produktion von Verbundmetall oder für die Ausführung der Rührung vom durch Partikel verstärkte Verbundmetall nach Anspruch 6, **dadurch gekennzeichnet, daß**, die Rührstation (2) beinhaltet einen Schmelztiegel (11), [u1] Einlass (23) für das Metall- oder Metalllegierungsmaterial, das geschämt wird, Matrixmaterialbehälter (24), Verstärkungsmaterialeinlass (25), Schaumpulvereinlass (22), beschützenden Gaseinlass (14) und einen Rührmechanismus (27) zusammen mit einem Oberrührdeckel (6), Kneten- und Einmischungsapparat (18); wo beschützende Gas (N₂ oder Argon) kontinuierlich auf den Schmelztiegel (11) gesprüht wird.

8. Ein Gerät für die Produktion von Verbundmetall oder für die Ausführung der Rührung vom durch Partikel verstärkte Verbundmetall nach Ansprüche 6 oder 7, **dadurch gekennzeichnet, daß** das Verstärkungsmaterial, Matrixmaterial und Schaumpulverzugaben (25, 23, und 22) sind sichergestellt durch automatische Kontrolleinheit, nach der Information erhalten von den Sensoren (19 und 20).

9. Ein Gerät für die Produktion von Verbundmetall oder für die Ausführung der Rührung vom durch Partikel verstärkte Verbundmetall nach Ansprüche 6 oder 7, **dadurch gekennzeichnet, daß** das Material im Innern des Metall- oder Metalllegierungsbehälters (24), das geschäumt oder zum durch Partikel verstärkten Verbundmetall umgewandelt wird, ist unterbrochen in kleine Teilchen.

10. Ein Gerät für die Produktion von Verbundmetall oder für die Ausführung der Rührung vom durch Partikel verstärkte Verbundmetall nach Ansprüche 6 oder 7, **dadurch gekennzeichnet, daß** das Material im Innern des Metall- oder Metalllegierungsbehälters (24), das geschäumt oder zum durch Partikel verstärkten Verbundmetall umgewandelt wird, ist vorbereitet und verarbeitet in Partikel- oder Pulverform ausgebildet von Metallplatte, Barren- oder wiederverwerteten Materiale.

11. Ein Gerät für die Produktion von Verbundmetall oder für die Ausführung der Rührung vom durch Partikel verstärkte Verbundmetall nach Ansprüche 6 oder 7, **dadurch gekennzeichnet, daß** das Metall oder Metalllegierungsmaterial, das geschäumt oder zum durch Partikel verstärkten Verbundmetall umgewandelt wird, kann bestehen aus Aluminium, Kupfer, Titanium, Nickel oder andere Metalle.

12. Ein Gerät für die Produktion von Verbundmetall oder für die Ausführung der Rührung vom durch Partikel verstärkte Verbundmetall nach Ansprüche 6 oder 7, **dadurch gekennzeichnet, daß** das Kneten- und Einmischungsapparate (18) operiert werden durch Rührmechanismus (27), Drucksensoren (20) und Temperatursensoren (19) im Rührmechanismus (27) befindlich sind, daß der Einmischungsprozedur durchgeführt ist von automatischer Kontrolleinheit in einer kontrollierten Weise nach der Viskosität / Stabilisation und Temperaturinformation erhalten von Druck- und Temperatursensoren (19 und 20).

13. Ein Gerät für die Produktion von Verbundmetall oder für die Ausführung der Rührung vom durch Partikel verstärkte Verbundmetall nach Ansprüche 6 oder 7, **dadurch gekennzeichnet, daß** die Mischung gehalten wird an einem halbfesten Aggregatszustand im Verlauf der Einmischungsperiode, und falls die Viskosität gering ist (vom halbfesten zum flüssigen Aggregatszustand) die Viskosität ist erhöht durch Zugabe von Metall oder Metalllegierung, die geschäumt wird, und falls die Viskosität hoch ist, kein zusätzliches Metall ist hinzugefügt zur Mischung aber der Einmischungsprozess ist weitergeführt und die Druck- und Temperatursensoren (19 und 20), die von Kontrolleinheit kontrolliert sind, sind verwendet um festzustellen, ob die Mischung an einem halbfesten Aggregatszustand ist und der Einmischungsprozess ist durchgeführt wieder von Befehle, die zum Rührer- und Metallhinzufügungsmechanismus gesendet sind von der Kontrolleinheit.

14. Ein Gerät für die Produktion von Verbundmetall oder für die Ausführung der Rührung vom durch Partikel verstärkte Verbundmetall nach Ansprüche 6 oder 7, **dadurch gekennzeichnet, daß** das Kneten- und Einmischungsapparat (18) verbunden zum Rührmechanismus (27) durchführt eine Bewegung (27b) auf und ab und eine radiale Bestrebung (27a) und die Rührzeiten und der Auswahl der Rührarmen, deren Anfügung und Demontage sind vom elektronischen System kontrolliert.

15. Ein Gerät für die Produktion von Verbundmetall oder für die Ausführung der Rührung vom durch Partikel verstärkte Verbundmetall nach Ansprüche 6 oder 7, **dadurch gekennzeichnet, daß** die Enden des Kneten- und Einmischungsapparats (18) verbunden zum Rührmechanismus (27) können flach, spiral oder durchlöchert sein.

16. Ein Gerät für die Produktion von Verbundmetall oder für die Ausführung der Rührung vom durch Partikel verstärkte Verbundmetall nach Ansprüche 6 oder 7, **dadurch gekennzeichnet, daß** die Löcher in Enden der durchlöcherten Kneten- und Einmischungsapparate (18) können runde, quadratische, elliptische, rechteckige oder polygonal geometrische Formen haben und jedes Loch kann in derselben oder in verschiedenen Größen stehen.

17. Ein Gerät für die Produktion von Verbundmetall oder für die Ausführung der Rührung vom durch Partikel verstärkte Verbundmetall nach Ansprüche 6 oder 7, **dadurch gekennzeichnet, daß** das Material vom Kneten- und Einmischungsapparat (18) mit einem hochtemperaturwiderstandsfähigen Material beschichtet ist wie Graphit oder Keramik.

18. Ein Gerät für die Produktion von Verbundmetall oder für die Ausführung der Rührung vom durch Partikel verstärkte Verbundmetall nach Ansprüche 6 oder 7, **dadurch gekennzeichnet, daß** die Oberfläche vom Kneten- und Einmischungsapparat (18) beschichtet ist mit einer Mischung vorbereitet vom Silizium, Karbidpulver und Kolloidsilizium.

19. Ein Gerät für die Produktion von Verbundmetall oder für die Ausführung der Rührung vom durch Partikel verstärkte Verbundmetall nach Ansprüche 6 oder 7, **dadurch gekennzeichnet, daß** es besteht aus einer Vielfalt von Schmelztiegel (11), die beweglich sind, sodaß sie der Reihe nach verwendet werden können, um andauernd eine halbfeste Fertigmischung sicherzustellen, daß der leere Schmelztiegel (11) nach vorne aus der Rührstation (2) verschoben ist, ein neuer Schmelztiegel (11) ist geschoben in den Platz, der nächste mit der Mischung aufgeladene Schmelztiegel, der in die Warteschlange verschoben ist, wird mit Gussformen ausgerichtet und daß diese Prozedur wiederholt ist, um andauernd Fertigmischungen sicherzustellen.

20. Ein Gerät für die Produktion von Verbundmetall oder für die Ausführung der Rührung vom durch Partikel verstärkte Verbundmetall nach Ansprüche 6 oder 7, **dadurch gekennzeichnet, daß** Unterteile des Schmelztiegels (11) offen stehen, daß der vordere Teil der beweglichen Gussform auch funktioniert wie die Sitzfläche des Schmelztiegels (25), und daß der besagte Unterteil an einer geschlossenen Position ist im Verlauf der Rührprozesse.

21. Ein Gerät für die Produktion von Verbundmetall oder für die Ausführung der Rührung vom durch Partikel verstärkte Verbundmetall nach Ansprüche 6 oder 7, **dadurch gekennzeichnet, daß** bewegliche Gussformen versetzt sind auf ein Gussformbett (9) hergestellt von Feuerfestziegeln, die sich erstrecken vom Einlassdeckel (4) der Gussform in den Ausflussdeckel der Gussform.

22. Ein Gerät für die Produktion von Verbundmetall oder für die Ausführung der Rührung vom durch Partikel verstärkte Verbundmetall nach Ansprüche 6 oder 7, **dadurch gekennzeichnet, daß** das Schmelztiegelmaterial (11) SiC, Al₂O₃ oder Graphit ist.

23. Ein Gerät für die Produktion von Verbundmetall oder für die Ausführung der Rührung vom durch Partikel verstärkte Verbundmetall nach Ansprüche 6 oder 7, **dadurch gekennzeichnet, daß** die Sitzfläche des Schmelztiegels (12) hergestellt ist aus hochtemperaturwiderstandsfähigem und hochwärmeleitfähigem Material, vorzugsweise aus Graphit.

24. Ein Gerät für die Produktion von Verbundmetall oder für die Ausführung der Rührung vom durch Partikel verstärkte Verbundmetall nach Ansprüche 6 oder 7, **dadurch gekennzeichnet, daß** der Behälter (13) hergestellt ist aus hochtemperaturwiderstandsfähigem und schwachwärmeleitfähigem Material.

25. Ein Gerät für die Produktion von Verbundmetall oder für die Ausführung der Rührung vom durch Partikel verstärkte Verbundmetall nach Ansprüche 6 oder 7, **dadurch gekennzeichnet, daß** der Behälter (13) aus Leichtbeton oder Keramikschaum ist.

26. Ein Gerät für die Produktion von Verbundmetall oder für die Ausführung der Rührung vom durch Partikel verstärkte Verbundmetall nach Anspruch 6, **dadurch gekennzeichnet, daß** ein Fanmechanismus (16) vorhanden ist auf dem Gussformausgangsdeckel, sodaß das Schaummaterial, das aus dem Schmelzofen herausgenommen ist, abgekühlt werden kann.

## Revendications

1. Procédé continu de production de mousse métallique composite, **caractérisé en ce qu'** 'il comprend les étapes suivantes,
• Les moules mobiles (8) et les poudres de renfort sont soumis à un préchauffage dans la section de préchauffage (1) du four ayant une température de 40 à 60 ° C en dessous de la température de fusion du métal ou de l'alliage métallique qui doit être converti en mousse ,
• Le creuset (11) contenant du métal ou un alliage métallique utilisé pour produire de la mousse, est délivré dans la section d'agitation (2) ayant une température de 100 à 300°C supérieure à la température de fusion du métal ou de l'alliage métallique qui doit être transformée en mousse et le métal ou l'alliage métallique à mousser est ajouté dans ledit creuset,
• En attendant la température du métal ou de l'alliage de métal qui doit être transformé en mousse présente à l'intérieur du creuset (11) pour augmenter et atteindre la plage de température dans laquelle le métal ou l'alliage de métal devient semi-solide,
• En prenant les moules mobiles (8) du couvercle d'entrée du moule (4) et en les déplaçant dans la section de préchauffage (1) et en amenant la température à la température de la section de préchauffage (1),
• Lorsque le matériau à l'intérieur du creuset (11) est ramolli et écrasé, le matériau renforcé qui a été passé par préchauffage est ajouté dans le creuset (11) par l'entrée de matériau renforcé (25),
• Afin de s'assurer que le métal ou l'alliage métallique à mousser, à l'intérieur du creuset (11), est maintenu à une plage de température semi-solide, si la viscosité du mélange (d'un semi-solide à un liquide) est faible selon à l'information obtenue à partir des capteurs de pression et de température (19 et 20), du métal ou de l'alliage de métal à mousser est ajouté au mélange pour augmenter la viscosité du mélange, **pendant ce temps, il n'a plus de matériau de renforcement ajouté;** et si la viscosité est élevée, la procédure
d'agitation est poursuivie sans addition de métal ou d'alliage métallique au mélange, en maintenant le mélange à semi-solide et en poursuivant jusqu'à ce que l'addition du matériau de renforcement soit terminée.
• Une fois que le mélange a été préparé à la quantité souhaitée, on ajoute dans le mélange à travers l'entrée de poudre moussante (22) la poudre moussante trouvée à l'intérieur du récipient de poudre moussant (21) et la procédure d'agitation est effectuée rapidement et en ce moment, métal ou l'alliage de métal continue d'être ajouté dans le mélange,
• Lorsqu'un mélange homogène a été fourni, le moule mobile est décalé et le fond du creuset (11) est ouvert et le mélange est poussé par un piston de poussée (17) depuis le fond du creuset (11) et transféré vers la cavité du moule mobile (8)
• Lorsque le mélange est poussé par le piston (17), le mélange est déplacé à une vitesse rapide constante dans le roulement de moule (9) au moyen d'une tige-poussoir (15) et le mélange remplit la cavité du moule mobile,
• Le moule mobile (8) est introduit dans la section moussante (3) ayant une température de 50 à 70°C supérieure à la température de fusion du métal ou alliage métallique à mousser,
• Lorsque le temps d'attente en fonction de la quantité du mélange est rempli, la tige-poussoir (15) pousse le couvercle de sortie (5) du moule (8) et le mélange est retiré du four,
Le matériau en mousse à l'intérieur du moule est rapidement refroidi au moyen de ventilateurs de refroidissement (16).

2. Procédé d'agitation de métal composite renforcé par des particules; **caractérisé en ce que**;
• Les poudres de renfort sont préchauffées à la section de préchauffage (1) et sont amenées à traiter les températures,
• La section de préchauffage (1) du four est portée à une température de 40 à 60°C en dessous de la température de fusion du métal ou de l'alliage de métal qui doit être transformé en métal composite renforcé par des particules,
• Le creuset (11) contenant du métal ou un alliage métallique utilisé pour produire une production de métal composite renforcé par des particules est amené dans la section d'agitation (2) du four et la température de la section d'agitation (2) est de 100 à 300°C supérieure à la fusion température du métal ou de l'alliage métallique utilisé pour produire la production de métal composite,
• Le métal ou l'alliage métallique utilisé pour produire une production de métal composite à l'intérieur du creuset (11) situé à la section d'agitation (2) est maintenu jusqu'à sa température
est augmentée à la plage de température dans laquelle ledit métal ou alliage métallique est à semi-solide,
• Lorsque le matériau à l'intérieur du creuset (11) est ramolli et écrasé, le matériau renforcé qui a été passé par préchauffage est ajouté dans le creuset (11) par l'entrée de matériau renforcé (25),
• Afin de s'assurer que le matériau, à l'intérieur du creuset, est maintenu à une température semi-solide, lorsque la température dépasse la température semi-solide, le métal ou l'alliage métallique utilisé pour produire du métal composite est ajouté au creuset (11) ou l'addition du métal ou de l'alliage de métal, est effectuée par une unité de commande automatique selon les informations obtenues à partir des capteurs de pression (20), la viscosité du mélange est contrôlée par addition de métal ou d'alliage métallique selon les informations obtenues à partir de la pression et des capteurs de température (19 et 20), afin de conserver le mélange à semi-solide, si la viscosité du mélange est faible en métal ou
un alliage métallique utilisé pour produire du métal composite est ajouté au mélange afin d'augmenter la viscosité du mélange et si la viscosité du mélange est élevée, la procédure d'agitation est poursuivie
sans ajouter de métal au mélange, et si la température du mélange augmente, mais la viscosité diminue, le matériau de renforcement n'est pas ajouté au mélange mais seul du métal ou de l'alliage de métal est ajouté.
• Le mélange est vérifié s'il est à semi-solide ou non en déterminant au moyen des capteurs de pression et de température (19 et 20) commandés par l'unité de commande, et à nouveau l'état semi-solide est assuré par les commandes soumises à l'agitateur et mécanisme d'addition métallique.
• Une fois le matériau de renforcement ajouté, le procédé d'agitation s'effectue en déplaçant les agitateurs vers le haut et vers le bas et en même temps les agitateurs se déplacent à l'intérieur du creuset (11) radialement ou elliptiquement ou en forme de zigzag en changeant d'emplacement sur l'orbite afin de porter sortir le processus de pétrissage et d'agitation ensemble jusqu'à ce que le matériau soit homogénéisé au moyen d'agitateurs suite à l'addition de matériau de renforcement,
• Lorsqu'un mélange homogène est obtenu, le mélange composite à l'intérieur du creuset (11) est retiré et versé dans des moules, de sorte qu'une production de matériau composite renforcée par des particules est obtenue au moyen d'un procédé de coulée ou de production.

3. Procédé selon les revendications 1 et 2, **caractérisé en ce que**: le matériau de renforcement est le SiC, le B₄C, l'Al₂O₃, le TiC et d'autres carbures, oxydes, nitrures et céramique.

4. Procédé selon la revendication 1 ou 2, **caractérisé en ce que** l'appareil de pétrissage et d'agitation (18) qui effectue le traitement de pétrissage et d'agitation en même temps avec le mélange homogène du matériau est déplacé vers le haut et vers le bas, et en même temps, radialement, elliptique dans le creuset (11) ou changements sur une orbite zig zag.

5. Procédé continu de production de mousse métallique composite selon la revendication 1, **caractérisé en ce que** la poudre moussante est TiH₂ et CaCO₃.

6. Dispositif pour produire du métal composite ou pour effectuer une agitation métallique composite renforcée par des particules, **caractérisé en ce que**: il comprend trois sections, la section de préchauffage (1), la section d'agitation (2) et la section de mousse (3), chaque section (1, 2, 3) étant chauffée avec des groupes de résistance séparés (7); dans lequel les contrôles de température peuvent être effectués séparément; et dans lequel la température de la section de préchauffage (1) du four est à une température inférieure à 40 à 60°C, la température de la section de mousse (3) est à une température supérieure à 50 à 70°C de la température de fusion du métal ou de l'alliage métallique à mousser, et dans lequel la température de la section d'agitation (2) est de 100 à 300°C supérieure à la température de fusion du métal ou de l'alliage métallique à mousser.

7. Dispositif pour produire du métal composite ou pour effectuer une agitation métallique composite renforcée par des particules selon la revendication 6, **caractérisée en ce que**: la section d'agitation (2) comprend un creuset (11), [u1] une entrée (23) pour le matériau en métal ou en alliage métallique à mousser, le récipient de matériau matriciel (24), l'entrée de matériau de renforcement (25), l'entrée de poudre moussante (22), l'entrée de gaz de protection (14) et un mécanisme d'agitation (27) avec un couvercle d'agitation supérieur (6), un appareil de pétrissage et d'agitation (18); dans lequel le gaz protecteur (N₂ ou argon) est pulvérisé en continu sur le creuset (11).

8. Dispositif pour produire du métal composite ou pour effectuer une agitation métallique composite renforcée par des particules selon la revendication 6 ou 7, **caractérisée en ce que**: le matériau de renforcement, le matériau de matrice et les ajouts de poudre moussante (25, 23 et 22) sont fournis par l'unité de commande automatique, selon les informations obtenues à partir des capteurs (19 et 20).

9. Dispositif pour produire du métal composite ou pour effectuer une agitation métallique composite renforcée par des particules selon la revendication 6 ou 7, **caractérisée en ce que**: le matériau à l'intérieur du récipient en métal ou en alliage métallique (24) qui doit être moussé ou transformé en composite renforcé par des particules, est divisé en petits morceaux.

10. Dispositif pour produire du métal composite ou pour effectuer une agitation métallique composite renforcée par des particules selon la revendication 6 ou 7, **caractérisée en ce que**: le matériau à l'intérieur du récipient en métal ou en alliage métallique (24) qui doit être expansé ou transformé en composite renforcé par des particules est préparé et traité sous forme de particules ou de poudre fabriqué à partir de plaques de métal, de lingots ou de matériaux recyclés.

11. Dispositif pour produire du métal composite ou pour effectuer une agitation métallique composite renforcée par des particules selon la revendication 6 ou 7, **caractérisée en ce que**: le matériau en métal ou en alliage métallique qui doit être expansé ou transformé en composite renforcé par des particules, peut être composé d'aluminium, de cuivre, de titane, de nickel ou d'autres métaux.

12. Dispositif pour produire du métal composite ou pour effectuer une agitation métallique composite renforcée par des particules selon la revendication 6 ou 7, **caractérisée en ce que**: l'appareil de pétrissage et d'agitation (18) est actionné par le mécanisme d'agitation de pétrissage (27), les capteurs de pression (20) et les capteurs de température (19) sont situés à l'intérieur du mécanisme d'agitation (27), que l'agitation est effectuée par l'unité de commande automatique de manière contrôlée en fonction de l'information de viscosité / stabilité et température obtenue à partir des capteurs de pression et de température (19 et 20).

13. Dispositif pour produire du métal composite ou pour effectuer une agitation métallique composite renforcée par des particules selon la revendication 6 ou 7, **caractérisée en ce que**: le mélange est maintenu à semi-solide pendant la période d'agitation, et si la viscosité est faible (d'un semi-solide à un liquide), la viscosité augmente en ajoutant du métal ou un alliage métallique à mousser et si la viscosité est élevée pas de supplément du métal est ajouté au mélange mais le processus d'agitation est poursuivi et les capteurs de pression et de température (19 et 20) contrôlés par l'unité de commande sont utilisés pour déterminer si le mélange est à semi-solide et le processus d'agitation est repris par les commandes envoyées à l'agitateur et au mécanisme d'addition métallique par l'unité de commande.

14. Dispositif pour la production de métal composite ou pour la réalisation de composite renforcé de particules agitation de métal selon la revendication 6 ou 7, **caractérisée en ce que**: l'appareil de pétrissage et d'agitation (18) relié au mécanisme d'agitation (27) effectue un mouvement ascendant et descendant (27b) et un mouvement radial (27a), les temps d'agitation et la sélection des tiges d'agitation, leur fixation et leur démontage sont contrôlés par le système électronique.

15. Dispositif pour produire du métal composite ou pour effectuer une agitation métallique composite renforcée par des particules selon la revendication 6 ou 7, **caractérisée en ce que**: les extrémités de l'appareil de pétrissage et d'agitation (18) relié au mécanisme d'agitation (27) peuvent être plates, en spirale ou perforées.

16. Dispositif pour produire du métal composite ou pour effectuer une agitation métallique composite renforcée par des particules selon la revendication 6 ou 7, **caractérisée en ce que**: les trous dans les extrémités de l'appareil de pétrissage et d'agitation perforées (18) peuvent avoir des formes géométriques rondes, carrées, elliptiques, rectangulaires ou polygonales et chaque trou peut être de la même taille ou peut être de différentes tailles.

17. Dispositif pour produire du métal composite ou pour effectuer une agitation métallique composite renforcée par des particules selon la revendication 6 ou 7, **caractérisée en ce que**: le matériau de l'appareil de pétrissage et d'agitation (18) est revêtu d'un matériau résistant aux hautes températures tel que le graphite ou la céramique.

18. Dispositif pour produire du métal composite ou pour effectuer une agitation métallique composite renforcée par des particules selon la revendication 6 ou 7, **caractérisée en ce que**: la surface de l'appareil de pétrissage et d'agitation (18) est revêtue d'un mélange préparé à partir de silicium, de poudre de carbure et de silice colloïdale.

19. Dispositif pour produire du métal composite ou pour effectuer une agitation métallique composite renforcée par des particules selon la revendication 6 ou 7, **caractérisée en ce qu'** 'elle comprend une pluralité de creusets (11) qui peuvent être déplacés de sorte qu'ils peuvent être utilisés en séquence pour fournir un semi-solide prêt à consommer en permanence, que le creuset vide (11) soit poussé vers l'avant hors de la section d'agitation (2), un nouveau creuset (11) est mis en place, le prochain creuset chargé avec le mélange est poussé dans la file d'attente pour être aligné avec les moules et que cette procédure est répétée pour fournir des mélanges prêts en continu.

20. Dispositif pour produire du métal composite ou pour effectuer une agitation métallique composite renforcée par des particules selon la revendication 6 ou 7, **caractérisée en ce que**: les parties inférieures des creusets (11) sont ouvertes, que la section avant du moule mobile fonctionne également comme fond de creuset (25), et que ladite partie inférieure est en position fermée pendant les processus d'agitation.

21. Dispositif pour produire du métal composite ou pour effectuer une agitation métallique composite renforcée par des particules selon la revendication 6 ou 7, **caractérisée en ce que**: les moules mobiles sont déplacés sur un lit de moule (9) en briques feuillues qui s'étendent depuis le couvercle d'entrée (4) du moule jusqu'au couvercle de sortie du moule.

22. Dispositif pour produire de la mousse métallique composite et pour le métal composite à agitation renforcée par des particules selon la revendication 6 ou 7, **caractérisé en ce que** le matériau du creuset (11) est du SiC, Al₂O₃ ou du graphite.

23. Dispositif pour produire de la mousse métallique composite et pour le métal composite agité renforcé par des particules selon la revendication 6 ou 7, **caractérisé en ce que** le fond du creuset (12) est constitué d'un matériau résistant aux hautes températures et à haute température, de préférence du graphite.

24. Dispositif pour produire de la mousse métallique composite et pour le métal composite à agitation renforcée par des particules selon la revendication 6 ou 7, **caractérisé en ce que** le récipient (13) est constitué d'un matériau résistant aux hautes températures et à faible chaleur conductrice.

25. Dispositif pour produire de la mousse métallique composite et pour le métal composite à agitation renforcée par des particules selon les revendications 6 et 7, **caractérisé en ce que** le récipient (13) est du béton gazeux ou de la mousse céramique.

26. Dispositif pour produire une mousse métallique composite ou pour un métal composite renforcé par des particules agitées selon la revendication 6, **caractérisé en ce qu'** 'un mécanisme de ventilateur (16) est présent sur le couvercle de sortie du moule de sorte que le matériau en mousse sorti du four puisse être refroidi.
